

## UNITED STATES PATENT OFFICE

1,928,652

PROCESS OF MAKING MIXED ESTERS OF  
CELLULOSECarl J. Malm and Charles R. Fordyce, Rochester,  
N. Y., assignors to Eastman Kodak Company,  
Rochester, N. Y., a corporation of New YorkNo Drawing. Application July 28, 1931  
Serial No. 553,633

18 Claims. (Cl. 260—101)

This invention relates to the making of various multi-acylated cellulose derivatives by introducing organic acid radicals into higher fatty acid esters of cellulose, (both simple and mixed) 5 which have been partially hydrolyzed.

An object of our invention is to provide a process for making the mixed esters of cellulose in which the proportions of acyl radicals may be controlled.

10 Another object of our invention is to provide a process of making cellulose esters having distinctive properties which adapt them for particular uses, some of which uses are not usually considered as adapted to the employment of esters of cellulose.

Hitherto the production of the mixed esters of cellulose has been either by esterifying cellulose with an acylating mixture which contributes a plurality of organic acid radicals to the cellulose or by esterifying an acetone-soluble cellulose acetate as disclosed, for example, in U. S. Patent No. 1,693,048 to Clarke and Malm. The former method does not admit of as accurate and precise control as may sometimes be desirable in 20 commercial manufacture. The latter process is not as well suited as the herein described process for the production of certain mixed esters of cellulose which do not contain the acetyl group such as cellulose propionate-stearate for example.

We have found that our process permits of the production of a multitude of mixed esters of cellulose in many cases varying only by a few percent in the proportions of organic acid radicals present. We have found that the partially hydrolyzed esters of cellulose containing higher acyl radicals are eminently suited for further esterification to form multi-acylated esters of cellulose.

We have found that by reason of the control of 40 the content of acyl groups possible in the hydrolysis of the higher esters of cellulose, precise regulation of the type of mixed esters of cellulose resulting from our process is facilitated. Some of the esters which, when partially hydrolyzed are 45 suitable for further esterification are cellulose propionate, cellulose butyrate, cellulose acetate-propionate and cellulose acetate-butyrate, as well as esters containing higher acyl radicals such as cellulose laurate, cellulose stearate, cellulose acetate-laurate and cellulose acetate-stearate. The hydrolysis of the mixed esters of cellulose may be carried out by the method of Malm and Fletcher application, serial No. 551,546, which discloses that the hydrolysis may be carried out in 55 an aqueous organic acid solution for example, at

about 100° F. The simple esters may be hydrolyzed by a like method or by any method disclosed in the prior art.

We have found that the partially hydrolyzed higher esters of cellulose are susceptible of further esterification by (1) fatty acid anhydrides, 60 (2) fatty acids together with an impeller or (3) fatty acid chlorides. The esterification by means of a fatty acid anhydride may be carried out either in a solvent reaction mixture or by fibrous acylation in a liquid such as toluene which is a non-solvent both for the hydrolyzed ester and for the final product. Various suitable liquids such as, for example, monochloracetic acid, alkoxy acetic acid, ethylene chloride, etc. or, in some 65 cases, the acid corresponding to the anhydride employed or even a different organic acid may be used as the solvent when esterifying in a solvent reaction mixture.

The following examples are illustrative of the 70 application of our invention to the production of mixed esters of cellulose:

## Example I

100 lbs. of cellulose propionate which has been 80 hydrolyzed to a propionyl content of about 45%, is placed in a reaction bath containing 400 lbs. of stearic acid, 400 lbs. of chloracetic anhydride, 800 lbs. of chloracetic acid and a small amount of a catalyst, such as magnesium perchlorate. 85 The mass is heated to about 65° C. for about 6 hours. The ester obtained may then be isolated from the reaction mixture by precipitating in methyl alcohol.

The product formed is cellulose propionate- 90 stearate which is acetone-soluble and is also soluble in hot mineral oil of medium viscosity, which solution upon cooling forms a jell of the consistency of heavy grease.

## Example II

100 lbs. of cellulose propionate containing about 45% propionyl is placed in a reaction bath containing 300 lbs. of glacial acetic acid, 250 lbs. of acetic anhydride and a small amount of sulfuric acid. The mass is maintained at about 100 32° C. for several hours. The resulting ester may then be precipitated in dilute acetic acid according to the method disclosed in Malm application No. 553,647.

The resulting product is cellulose-acetate-propionate which is soluble in acetone, ethylene chloride and methyl acetate.

If desired, the temperature may be maintained at 48°-66° C. in which case, the time and the 110

amounts of acid and anhydride may be reduced. In such case, a buffer such as sodium acetate, or some other alkali metal salt may be added, if desired, to eliminate any danger of degradation.

*Example III*

100 lbs. of cellulose butyrate having about 50% butyryl content is placed in a reaction mixture containing 200 lbs. of stearic anhydride, 800 lbs. of ethoxy-acetic acid and a small amount of magnesium perchlorate. The mass is kept at about 65° C. for about 10 hours at the end of which time the resulting ester may be separated from its reaction mixture by pouring the latter with agitation into methyl alcohol. The cellulose butyrate-stearate formed is soluble in various hydrocarbons such as mineral oil, ligroin etc. as well as in vegetable oils such as castor oil.

*Example IV*

100 lbs. of cellulose acetate-butyrate having about a 35% acetyl and 12% butyryl content is placed in a reaction mixture containing 300 lbs. of lauric acid, 300 lbs. of ethoxy acetic anhydride, 600 lbs. of ethylene chloride and a small amount of magnesium perchlorate which is maintained at about 65° C. for about 10 hours. The resulting ester is isolated from its reaction mass by pouring with agitation into iso-propyl ether, the ester being thereafter washed with such ether. The resulting product is cellulose acetate-butyrate-laurate which is product soluble in acetone, benzene, toluene and chloroform.

*Example V*

100 lbs. of cellulose butyrate having about a 50% butyryl content which has been subjected to 100 hours hydrolysis is placed in a reaction mixture containing approximately 1500 lbs. of toluene, 150 lbs. of propionic anhydride and 40 lbs. of pyridine. The mixture is refluxed for 15-30 hours. The cellulose ester obtained is filtered off and washed. A cellulose propionate-butyrate is obtained.

*Example VI*

100 lbs. of cellulose acetate-propionate, having about a 30% acetyl and 12% propionyl content is placed in about 1500 lbs. of toluene. The moisture present is distilled off and a mixture of about 500 lbs. of stearic anhydride, 30 lbs. of p-toluenesulfo-chloride and 1500 lbs. of ligroin (B. P. 90-120° C.) is added. The mixture is refluxed for 15-30 hours, depending upon the speed of the reaction after which the cellulose ester may be filtered off and washed with hot water if desired. A cellulose acetate-propionate-stearate is obtained.

*Example VII*

100 lbs. of cellulose butyrate, having about a 50% butyryl content is placed in 300 lbs. of pyridine, and 400 lbs. of lauryl chloride in 400 lbs. of toluene is added. The mass is heated for 3-5 hours at about 50° C. or until complete acylation occurs. The cellulose butyrate-laurate obtained is separated from the reaction mass by pouring the latter with agitation into methyl alcohol. The ester is soluble in acetone, ethyl acetate, benzene and chloroform.

*Example VIII*

100 lbs. of cellulose butyrate having about a 50% butyryl content is placed in a reaction mix-

ture containing about 200 lbs. of stearic anhydride, 800 lbs. of ethylene chloride and a small amount of magnesium perchlorate. The mass is kept at about 65° C. for about 10 hours at the end of which time the resulting ester may be separated from its reaction mixture by pouring the latter with agitation into methyl alcohol. The cellulose butyrate-stearate formed is soluble in various hydrocarbons such as mineral oil, ligroin etc. as well as in vegetable oils such as castor oil.

As pointed out before, the esters of cellulose containing high radicals, such as lauryl, stearyl, palmityl, etc., when partially hydrolyzed, may be employed as the starting material for adding additional acyl groups according to the method disclosed by the above examples. However, it is preferred to start with the propionate or butyrate containing esters and substitute other groups therein.

If desired, a series of acylations, according to our process, may be employed to prepare esters having several different acyl radicals attached to the cellulose. For example, a hydrolyzed cellulose propionate may be esterified according to our process by which a butyrate group is added. This cellulose propionate-butyrate may then be hydrolyzed and the resulting hydrolyzed cellulose propionate-butyrate may then be esterified with the addition of a lauryl group. Thus, a cellulose propionate-butyrate-laurate may be formed. Still further hydrolysis and esterification is, of course, possible if the addition of still further groups is desired.

If desired, more than one group may be added to the hydrolyzed ester upon esterification. For example, hydrolyzed cellulose propionate may be esterified in a bath containing acetic anhydride and lauric acid or it may, for example, be esterified in a bath containing an impeller such as ethoxyacetic anhydride and a plurality of organic acids.

The catalysts which will promote acylation reactions are well known and need not be enumerated here. It is, of course, within the judgment of the skilled artisan to determine which of these acylation catalysts is most suitable for the particular esterification which he desires to carry out. The employment of any of the known catalysts for acylation in our process comes within the contemplation of our invention. The various solvents or non-solvents which may be employed in the esterification according to our process are also a matter of choice and the selection of a particularly well known solvent for carrying out the esterification of the hydrolyzed esters according to our process is within the scope of our invention.

The esters which are produced by our process may be employed for many and various uses, such as the forming of sheets or films, filaments for artificial silk, lacquers, lubricants, artificial leather, materials for moulding, waterproof coating or any other capacity in which cellulose esters have previously been employed. Many of the esters made according to our process have qualities which give them exceptional adaptability in this art, for example, some of these esters give films and filaments without employing plasticizers. However, compatible plasticizers such as triphenyl or tricresyl-phosphate, may be incorporated with the esters produced by our process when forming colloidized products therefrom.

Our esters may also be mixed with other cellulose esters, such as cellulose acetate or cellulose

nitrate and/or with other plastic materials such as gums, resins, waxes, heavy metal soaps, etc. They may also be employed for laminating or reinforcing glass, cellulose derivatives or other materials, especially when they are in sheet or layer form.

Other modifications of our process and other uses for the esters so produced which will occur to those skilled in the art also come within the contemplation of our invention.

It is to be understood that the term "higher organic" is employed herein to designate either radicals above acetyl in the number of carbon atoms or esters which contain such radicals.

15 What we claim as our invention is:

1. The process of producing a mixed ester of cellulose which comprises esterifying a partially hydrolyzed acyl ester of cellulose containing a higher aliphatic acid radical and 1-4 hydroxyl groups to every 24 carbon atom unit of cellulose.

2. The process of producing a mixed ester of cellulose which comprises esterifying a hydrolyzed acyl ester of cellulose containing the radical of a fatty acid higher than acetic and 1-4 hydroxyl groups to every 24 carbon atom unit of cellulose.

3. The process of producing a mixed ester of cellulose which comprises esterifying a hydrolyzed acyl ester of cellulose containing an aliphatic acid radical of 3-4 carbon atoms and 1-4 hydroxyl groups to every 24 carbon atom unit of cellulose.

4. The process of producing a mixed ester of cellulose which comprises treating a hydrolyzed acyl ester of cellulose containing a higher aliphatic radical and 1-4 hydroxyl groups to every 24 carbon atom unit of cellulose with an esterifying bath containing an aliphatic acid anhydride.

5. The process of producing a mixed ester of cellulose which comprises treating a hydrolyzed acyl ester of cellulose containing a higher aliphatic radical and 1-4 hydroxyl groups to every 24 carbon atom unit of cellulose with an esterifying bath containing an aliphatic acid anhydride and a catalyst.

6. The process of producing a mixed ester of cellulose which comprises treating a hydrolyzed acyl ester of cellulose containing an aliphatic acid radical of 3-4 carbon atoms and 1-4 hydroxyl groups to every 24 carbon atom unit of cellulose with an esterifying bath containing an aliphatic acid anhydride.

7. The process of producing a mixed ester of cellulose which comprises treating a hydrolyzed acyl ester of cellulose containing an aliphatic acid radical of 3-4 carbon atoms and 1-4 hydroxyl groups to every 24 carbon atom unit of cellulose with an esterifying bath containing an aliphatic acid anhydride and a catalyst.

8. The process of producing a mixed ester of cellulose which comprises esterifying a hydrolyzed acyl ester of cellulose selected from the group consisting of cellulose propionate, cellulose butyrate, cellulose acetate-propionate and cellulose-acetate butyrate and 1-4 hydroxyl groups to every 24 carbon atom unit of cellulose.

9. The process of producing a mixed ester of cellulose which comprises treating a hydrolyzed acyl ester of cellulose selected from the group consisting of cellulose propionate, cellulose butyrate, cellulose acetate-propionate and cellulose acetate-butyrate and 1-4 hydroxyl groups to every 24 carbon atom unit of cellulose with an esterifying bath containing an aliphatic acid anhydride.

75 10. The process of producing a mixed ester of

cellulose which comprises treating a hydrolyzed acyl ester of cellulose containing a higher aliphatic radical and 1-4 hydroxyl groups to every 24 carbon atom unit of cellulose with a bath containing an esterifying agent selected from the group consisting of a fatty acid anhydride, a fatty acid and a fatty acid chloride.

80

11. The process of producing a mixed ester of cellulose which comprises treating a hydrolyzed acyl ester of cellulose containing a higher aliphatic radical and 1-4 hydroxyl groups to every 24 carbon atom unit of cellulose with an esterifying bath containing a fatty acid anhydride and an organic liquid which is at least a solvent for the anhydride.

85

12. The process of producing a mixed ester of cellulose which comprises treating a hydrolyzed acyl ester of cellulose containing a higher aliphatic radical and 1-4 hydroxyl groups to every 24 carbon atom unit of cellulose with an esterifying bath containing a fatty acid and an organic liquid which is at least a solvent for the acid.

95

13. The process of producing a mixed ester of cellulose which comprises treating a hydrolyzed acyl ester of cellulose containing a higher aliphatic radical and 1-4 hydroxyl groups to every 24 carbon atom unit of cellulose with an esterifying bath containing a fatty acid chloride and an organic liquid which is at least a solvent for the chloride.

100

14. The process of producing a mixed ester of cellulose which comprises treating a hydrolyzed acyl ester of cellulose containing a higher aliphatic radical and 1-4 hydroxyl groups to every 24 carbon atom unit of cellulose with an esterifying bath containing a fatty acid anhydride, a catalyst and an organic liquid which is at least a solvent for the anhydride.

110

15. The process of producing a mixed ester of cellulose which comprises treating a hydrolyzed acyl ester of cellulose containing a higher aliphatic radical and 1-4 hydroxyl groups to every 24 carbon atom unit of cellulose with an esterifying bath containing a fatty acid, a catalyst and an organic liquid which is at least a solvent for the acid.

120

16. The process of producing a mixed ester of cellulose which comprises treating a hydrolyzed acyl ester of cellulose containing a higher aliphatic radical and 1-4 hydroxyl groups to every 24 carbon atom unit of cellulose with an esterifying bath, containing a fatty acid chloride, a catalyst and an organic liquid which is at least a solvent for the chloride.

125

17. The process of producing a mixed ester of cellulose which comprises treating a hydrolyzed acyl ester of cellulose containing a higher aliphatic acid radical and 1-4 hydroxyl groups to every 24 carbon atom unit of cellulose with an esterifying bath comprising a fatty acid, an impeller for the esterification and a catalyst.

135

18. The process of producing a mixed ester of cellulose which comprises treating a hydrolyzed acyl ester of cellulose containing a higher fatty acid radical and 1-4 hydroxyl groups to every 24 carbon atom unit of cellulose with an esterifying bath comprising a fatty acid and an impelling agent for the esterification selected from the group consisting of chloracetic anhydride, ethoxycacetic anhydride and methoxycacetic anhydride.

140

145